

June 2, 1959

A. H. MATUSZAK ET AL

2,889,281

SYNTHETIC LUBRICATING COMPOSITION

Filed March 21, 1956

2 Sheets-Sheet 1

FIGURE - 1



June 2, 1959

A. H. MATUSZAK ET AL  
SYNTHETIC LUBRICATING COMPOSITION

2,889,281

Filed March 21, 1956

2 Sheets-Sheet 2



Alfred H. Matuszak  
Arnold J. Morway Inventors

By *EJ Brenner* Attorney

1

2,889,281

## SYNTHETIC LUBRICATING COMPOSITION

Alfred H. Matuszak, Westfield, and Arnold J. Morway, Clark, N.J., assignors to Esso Research and Engineering Company, a corporation of Delaware

Application March 21, 1956, Serial No. 572,953

6 Claims. (Cl. 252—49.6)

This invention relates to new and improved synthetic lubricating compositions having outstanding extreme pressure-resisting characteristics. Particularly, the invention relates to extreme pressure lubricating compositions which comprise blends of dialkyl esters of dicarboxylic acids, complex esters, and critical amounts of two polymerized alkyl silicones of different molecular weights.

To meet the exacting requirements of lubricating oils having utility for the lubrication of moving metal parts which are subjected to extremely high pressures and temperatures, it has been found necessary by the industry to develop lubricants with special properties. Generally, mineral lubricating oils, even when containing large amounts of the various known additive materials, have been found to be unsuccessful for the lubrication of turbo-jet and turbo-prop aviation engines. Generally, the prior art mineral lubricating oils have failed in this lubricating service because of lack of stability at high temperatures, lack of sufficient load-carrying properties or too great a change of viscosity with temperature.

This invention is concerned with synthetic lubricating oils having characteristics which make them eminently suitable for this use. The lubricating compositions described in detail below have been found to have good temperature-viscosity relationships and extreme pressure-resisting characteristics along with other desirable properties which enable them to meet stringent military specifications for this use. As was set out above, these new and improved synthetic lubricating compositions comprise blends of a dialkyl ester of a dicarboxylic acid, a complex ester formed from three ingredients: a branched chain alcohol, a dicarboxylic acid and a glycol, and critical amounts of two different polymerized alkyl silicones. As will be pointed out in detail below, the components of the compositions must be present within certain critical limitations.

The major component of the compositions of this invention is a dialkyl ester of a dicarboxylic acid. These esters conform to the following general formula:



In the formula R is a branched chain alkyl group containing from 6 to 10 carbon atoms. This alkyl group may be derived from secondary and/or primary alcohols such as isohexyl, secondary hexyl, 2-ethylbutyl, isoheptyl, secondary heptyl, isoctyl, capryl, 2-ethylhexyl, isononyl, isodecyl, and the like. To obtain a higher degree of thermal stability at high temperatures the esters of primary alcohols are preferred over the esters derived from secondary alcohols. Among the operable branched chain alcohols, the well known "Oxo" alcohols and the aldol condensation alcohols (2-ethylhexyl, 2-ethylbutyl) are preferred. The isoctyl alcohol obtained by the carbonylation of a C<sub>7</sub> olefin in the presence of a cobalt catalyst at elevated temperatures and pressures are especially preferred when adipic acid and/or azelaic acids are involved whereas 2-ethylhexyl alcohol is preferred where sebacic acid is employed.

2

The dicarboxylic acid which is esterified with the desired alcohol to prepare the diester may be selected from the group consisting of succinic, glutaric, adipic, pimelic, suberic, azelaic, and sebacic acids, with azelaic and sebacic acids being especially preferred. The formula given above covers the operable acids when n is from 2 to 8.

A complex ester component of the lubricating oil compositions of this invention is prepared by the interaction of a branched chain alcohol having from 6 to 10 carbon atoms (e.g., 2-ethyl hexanol, C<sub>8</sub> oxoalcohol), a dicarboxylic acid having from 4 to 10 carbon atoms (e.g. sebacic acid, adipic acid), and a glycol having from 4 to 12 carbon atoms (e.g., tetraethylene glycol). These complex esters conform to the following general formula:



In the formula above, R represents the alkyl groups of the branched chain alcohols and will contain from 6 to 10 carbon atoms. x is a number from 2 to 8 and z, is a number from 2 to 6.

The preparation of the complex ester involves methods known to the art and forms no part of the inventive concept. Briefly stated, these complex esters may be prepared in a one-step process by reacting the required molar proportions of the alcohol (2 moles), the glycol (1 mole), and the dicarboxylic acid (2 moles) together in the presence of a water entrainer and an esterification catalyst at temperatures of about 350° to 425° F., until the theoretical quantity of water is evolved. If desired, a two-step process may be employed. Two moles of a half-ester of the dicarboxylic acid and the alcohol may first be formed, followed by complete esterification of the half-ester with 1 mole of the glycol; or two moles of the dicarboxylic acid are reacted with one mole of the glycol to form a glycol dicarboxylic acid ester which is then completely esterified with the alcohol. Each method gives essentially the same product equivalent in all quality aspects.

The combination of the diester component and the complex ester component of the synthetic lubricating composition comprises the lubricating oil base. The proportions of the components may vary between relatively restricted ranges. For example, it has been found that from 80% to 99% by volume of the diester may be blended with from 1 to 20% by volume of the complex ester. More preferred, however, are blends containing from 92 to 97% by volume of the diester with from 3% to 8% by volume of the complex ester. Especially preferred and contemplated in the preferred embodiment of this invention is a composition containing about 96% by volume of the diester with 4% by volume of the complex ester.

To this base composition, there is added a minor amount of an antioxidant such as purified phenothiazine, phenyl-a-naphthylamine, n-butyryl p-amino phenol, 2,6-di-tert butyl-p-cresol, etc. The proportions used may vary between about 0.25 and 2 weight percent of the antioxidant. However, satisfactory oxidation resistance for most applications will be obtained by the use of about 1.0 weight percent of phenothiazine.

The extreme pressure characteristics of the base composition referred to above have been found to be adequate to meet most lubricating requirements for present day turbo-jet engine applications. However, it has been found that the exceptionally severe conditions inherent in lubricating present and future type turbo-prop reduction gear assemblies (heavily loaded), and advanced design turbo-jet engines for supersonic aircrafts make it necessary to enhance the extreme pressure-resisting properties of this normally acceptable lubricant without increasing the overall viscosity and corrosivity of the lubricant. This has been accomplished by the instant inven-

tors by the inclusion in the base lubricant of specific amounts of a polymerized alkyl silicone of a specific molecular weight range. It should be emphasized that this has been done without adversely affecting the non-corrosivity of the base, a feat most difficult to accomplish with any other load carrying agent.

This polymerized alkyl silicone is a polymer of dimethyl silicone and has the formula:



This dimethyl silicone polymer is commercially available in several viscosity grades which represent batches of different molecular weights. It has been found that only the molecular weight polymers corresponding to from 3 to 20 centistokes viscosity at 25° C. are applicable to the formation of the improved synthetic lubricating compositions of this invention. As will be set out in detail below, when a polysilicone having a molecular weight above the 20 cs. viscosity range is used, there is an interaction or incompatibility between the silicone polymer and the diester and the complex esters which results in undesirable insolubility of the polymer. When a polysilicone of a molecular weight range below the 3 cs. viscosity grade is used, incompatibility is not a factor but the flash point of the resulting composition is lowered considerably. Furthermore, because of this high volatility (i.e. low flash point), excessive loss of the silicone ingredient could be expected during service should lower molecular weight or lower viscosity grade silicones be used. The loss experienced would of course depend also upon the concentration of silicone employed and upon the operating conditions to which the silicone blend is subjected.

The dimethyl silicone polymer is utilized in the formulation of the compositions of this invention in amounts varying between about 2 to about 25% by weight, with from about 5 to about 20% by weight being especially preferred to obtain the maximum load carrying ability. Because of the unusually high load carrying ability imparted to the blend by the dimethyl silicone, it has been found that 3 to 5% silicone will generally provide sufficient load carrying ability for most turbo applications. Furthermore, this range is reasonably economical.

When the dimethyl silicone polymers are blended with the base composition defined above, it has been found that contrary to the teaching of the prior art, the foaming characteristics of the composition are undesirably affected. Blends containing the dimethyl silicone polymer actually foam more than blends that do not contain this polymer. It has thus been found necessary to include in the finished lubricating composition minor amounts of a second polymer of dimethyl silicone of a molecular weight range corresponding to about 10,000 cs. or above at 25° C., with 60,000 to 200,000 cs. being especially preferred. Ordinarily, about 0.001 to 0.005 weight percent of this high molecular weight silicone has been found to eliminate the foam-forming tendency of the low molecular weight silicone. In certain instances, however, concentrations of about 0.05 to 0.1 weight percent have been required to impart desirable low-foaming characteristics to the finished lubricant blend.

The preferred lubricating compositions of this invention therefore comprise the following:

#### Parts by weight

|                                                       |           |
|-------------------------------------------------------|-----------|
| Base blend                                            | 100       |
| Diester, 92-97 vol. percent.                          |           |
| Complex ester, 3-8 vol. percent.                      | 0-2       |
| Anti-oxidant                                          |           |
| Dimethyl silicone polymer (3-20 cs./25° C.)           | 2-25      |
| Dimethyl silicone polymer (10,000-200,000 cs./25° C.) | 0.001-0.1 |
| Tricresyl phosphate                                   | 0-3       |

#### EXAMPLES

By admixing the components set out in detail below and heating with stirring to a temperature of about 150 to 180° F., lubricating compositions of the following ingredients were prepared:

[Ingredients, parts by weight]

|    |                                              | Blend 1 | Blend 2 | Blend 3 |
|----|----------------------------------------------|---------|---------|---------|
| 10 | Base blend                                   | 100     | 100     | 100     |
|    | Diisooctyl azelate, vol. percent.            | 95      | 97      | —       |
|    | 2-ethylhexyl sebacate, vol. percent.         | —       | —       | 38      |
| 15 | C <sub>8</sub> Oxo adipate, vol. percent.    | —       | —       | 57      |
|    | C <sub>10</sub> Oxo adipate, vol. percent.   | 5       | —       | —       |
|    | Complex ester A <sup>1</sup> , vol. percent. | —       | 3       | 5       |
|    | Complex ester B <sup>2</sup> , vol. percent. | 5       | 4       | 5       |
| 20 | Dimethyl silicone (10 cs./25° C.)            | 0.001   | 0.001   | 0.001   |
|    | Dimethyl silicone (60,000 cs./25° C.)        | —       | —       | 1       |
|    | Tricresyl phosphate                          | 1       | 1       | 1       |
|    | Phenothiazine                                | —       | —       | —       |

<sup>1</sup> Complex ester A: 2-ethylhexanol—sebacic acid—tetraethylene glycol—sebacic acid—2-ethylhexanol.

<sup>2</sup> Complex ester B: C<sub>8</sub> Oxo alcohol—adipic acid—tetraethylene glycol—adipic acid—C<sub>8</sub> Oxo alcohol.

These formulations are compared with current military specifications in Table I below:

Table I

|    | MIL-L-7808B and<br>MIL-L-25336<br>(USAF)<br>requirements                                                                                                                                                                                                                                                                                                                                                              | Blends                  |       |       |
|----|-----------------------------------------------------------------------------------------------------------------------------------------------------------------------------------------------------------------------------------------------------------------------------------------------------------------------------------------------------------------------------------------------------------------------|-------------------------|-------|-------|
|    |                                                                                                                                                                                                                                                                                                                                                                                                                       | 1                       | 2     | 3     |
| 30 | Viscosity at 210° F., cs.                                                                                                                                                                                                                                                                                                                                                                                             | 3.0 min.                | 3.36  | 3.35  |
|    | Viscosity at 100° F., cs.                                                                                                                                                                                                                                                                                                                                                                                             | 13.40                   | 12.76 | 12.78 |
| 35 | Viscosity at -65° F., cs.                                                                                                                                                                                                                                                                                                                                                                                             | 13,000 max.             | 8,085 | 8,315 |
|    | Pour point, ° F.                                                                                                                                                                                                                                                                                                                                                                                                      | <-75                    | <-80  | <-75  |
|    | Flash point, ° F.                                                                                                                                                                                                                                                                                                                                                                                                     | 350 min.                | 450   | 455   |
|    | Panel coking at 600° F., mg.                                                                                                                                                                                                                                                                                                                                                                                          | 100                     | 86    | 6     |
|    | Panel coking at 700° F., mg.                                                                                                                                                                                                                                                                                                                                                                                          | —                       | 409   | —     |
|    | Panel coking at 750° F., mg.                                                                                                                                                                                                                                                                                                                                                                                          | —                       | 1,750 | —     |
|    | "H" rubber swell, percent.                                                                                                                                                                                                                                                                                                                                                                                            | 12 to 35                | 21.4  | 25.2  |
| 40 | Foam Test:                                                                                                                                                                                                                                                                                                                                                                                                            |                         |       |       |
|    | Sequence 1                                                                                                                                                                                                                                                                                                                                                                                                            | 100-0                   | 5-0   | 10-0  |
|    | Sequence 2                                                                                                                                                                                                                                                                                                                                                                                                            | 25-0                    | 10-0  | 0-0   |
|    | Sequence 3                                                                                                                                                                                                                                                                                                                                                                                                            | 100-0                   | 10-0  | 0-0   |
|    | Copper corrosion, 50 hrs. at 450° F., mg.                                                                                                                                                                                                                                                                                                                                                                             | 3.0 max.                | 0.60  | 0.28  |
|    | Silver corrosion, 50 hrs. at 450° F., mg.                                                                                                                                                                                                                                                                                                                                                                             | 3.0 max.                | 0.42  | 0.32  |
| 45 | SOD lead corrosion, 1 hr. at 325° F. Mg.                                                                                                                                                                                                                                                                                                                                                                              | 30 max.                 | 8     | 1     |
|    | D-664 neut. no., mg. KOH/gm.                                                                                                                                                                                                                                                                                                                                                                                          | —                       | 0.10  | 0.22  |
|    | Oxidation corrosion stability, 72 hrs. at 347° F., mg./cm. <sup>2</sup>                                                                                                                                                                                                                                                                                                                                               |                         |       |       |
|    | Copper                                                                                                                                                                                                                                                                                                                                                                                                                | ±0.4                    | 0.01  | 0.04  |
|    | Magnesium                                                                                                                                                                                                                                                                                                                                                                                                             | ±0.2                    | 0.00  | 0.01  |
|    | Steel                                                                                                                                                                                                                                                                                                                                                                                                                 | ±0.2                    | 0.01  | 0.02  |
|    | Aluminum                                                                                                                                                                                                                                                                                                                                                                                                              | ±0.2                    | 0.04  | 0.01  |
|    | Silver                                                                                                                                                                                                                                                                                                                                                                                                                | ±0.2                    | 0.01  | 0.01  |
| 50 | Viscosity at 100° F. cs., after test.                                                                                                                                                                                                                                                                                                                                                                                 | —                       | 13.89 | 13.17 |
|    | Viscosity, percent change                                                                                                                                                                                                                                                                                                                                                                                             | -5 to +15               | 3.3   | 3.2   |
|    | Neut. number increase                                                                                                                                                                                                                                                                                                                                                                                                 | 2.0                     | 1.2   | 0.90  |
|    | Low temperature stability (-65° F.):                                                                                                                                                                                                                                                                                                                                                                                  |                         |       |       |
|    | Viscosity, cs., initial (35 mins.)                                                                                                                                                                                                                                                                                                                                                                                    | 13,000 max.             | 8,040 | 8,315 |
|    | Viscosity, cs. final (3 hrs. 37 mins.)                                                                                                                                                                                                                                                                                                                                                                                | 13,000 max.             | 8,256 | 8,315 |
|    | Viscosity, percent change                                                                                                                                                                                                                                                                                                                                                                                             | 6.0 max.                | 2.7   | 0.0   |
|    | Evaporation loss, percent at 400° F.                                                                                                                                                                                                                                                                                                                                                                                  | 50 max.                 | 22.1  | 26.1  |
| 60 | Ryder gear load, lbs./in., for MIL-L-7808B                                                                                                                                                                                                                                                                                                                                                                            | 1,700 min. <sup>1</sup> | 3,760 | 3,300 |
|    | Ryder gear load, lbs./in., for MIL-L-25336 (USAF)                                                                                                                                                                                                                                                                                                                                                                     | 2,800 min. <sup>1</sup> | 3,760 | 3,300 |
|    | SAE-SOD test load, lbs.                                                                                                                                                                                                                                                                                                                                                                                               | 550 <sup>2</sup>        | 1,275 | 1,300 |
| 65 | MIL-L-7808B Specification covers turbo-jet engine oils; MIL-L-25336 (USAF) Specification covers turbo-prop engine lubricants which are MIL-L-7808B type oils having increased load carrying ability.                                                                                                                                                                                                                  |                         |       |       |
|    | <sup>1</sup> SAE-SOD Test is not an MIL-L-7808B Specification requirement.                                                                                                                                                                                                                                                                                                                                            |                         |       |       |
|    | A lubricant giving a value of about 550 lbs. in this test will give about 1700 lbs./in. in the Ryder Gear Test. The test is performed in the SAE Lubricant Tester. The lubricant is run-in for two minutes at 50 lbs. load, then the load is manually increased 50 lbs. every 10 seconds until scuffing occurs. The load at which scuffing occurs is recorded and denotes the load carrying ability of the lubricant. |                         |       |       |

Because of the viscosity requirement of 13,000 cs. maximum at -65° F. in MIL-L-7808 and MIL-L-25336 Specification, the amount of the more viscous complex esters that can be incorporated in the lubricants of this

invention without exceeding this requirement will be limited. The actual amount employed will, of course, depend upon the viscosity level desired as well as the viscosities of the diester and complex ester components. The viscosities of the more desirable diesters range from 2.7 to 3.5 cs. at 210° F. and 5,000 to 10,000 cs. at -65° F. The viscosities of the complex esters are about 7 to 11 cs. at 210° F., and 100,000 to 500,000 cs. (extrapolated) at -65° F. The effect on these viscosities of varying the proportions of diester-complex ester base

10 inhibitor such as purified phenothiazine in the base oil blend of the compositions of this invention is necessary to prevent oxidative degradation during the life of the lubricant. The stabilizing effect of phenothiazine on the diester component is readily seen in the following examples. Its effect on the diester-complex ester bases of this invention is similar. It will be noted that with phenothiazine present, metal corrosion, solidification and acidity are held to a satisfactory level. Oxygen adsorption is also nil.

| Percent phenothiazine                                                                    | Di-2-ethylhexyl sebacate   |             | O <sub>8</sub> oxo adipate |             |
|------------------------------------------------------------------------------------------|----------------------------|-------------|----------------------------|-------------|
|                                                                                          | 0.0                        | 1.0         | 0.0                        | 1.0         |
| Corrosion/oxidation stability (250° F.) weight change, mg./cm. <sup>2</sup> , and color: |                            |             |                            |             |
| Copper                                                                                   | 0.0 magenta                | 0.06 purple | -7.3 copper                | 0.04 purple |
| Steel                                                                                    | 0.01 grey                  | 0.00 purple | 0.01 grey                  | 0.02 purple |
| Aluminum alloy                                                                           | 0.01 none                  | do          | do                         | 0.00 purple |
| Magnesium alloy                                                                          | -0.01 grey                 | do          | -6.0 etched                | 0.05 purple |
| Cadmium plated steel                                                                     | 1.48 badly etched          | 0.06 purple | -2.8 grey                  | 0.04 purple |
| Oil evaporated, percent                                                                  | 5.6                        | 0.88        | 7.4                        | 1.1         |
| Viscosity change at 100° F., percent                                                     | 87.5                       | 0.16        | Solid mass                 | 0.3         |
| Neut. number increase, mg. KOH/gm.                                                       | 75                         | 0.02        | 80                         | 0.1         |
| Oxidation rate—ml. O <sub>2</sub> absorbed in 4 successive 15 minute periods at 392° F.  | 250 <sup>+</sup> , -, -, - | 0, 0, 0     | 250 <sup>+</sup> , -, -, - | 0, 0, 0, 0  |

composition may be shown by the following series of blends.

| Blend                                                           | Viscosity, cs. at ° F. |        |
|-----------------------------------------------------------------|------------------------|--------|
|                                                                 | 210                    | -65    |
| A. 100% di-isooctyl azelate                                     | 3.35                   | 8,475  |
| B. 95% di-isooctyl azelate+5% complex sebacate A (10.3 cs.)     | 3.58                   | 9,250  |
| C. 90% di-isooctyl azelate+10% complex sebacate A (10.3 cs.)    | 3.79                   | 11,190 |
| D. 85% di-isooctyl azelate+15% complex sebacate A (10.3 cs.)    | 4.02                   | 13,540 |
| E. 80% di-isooctyl azelate+20% complex sebacate A (10.3 cs.)    | 4.25                   | 16,350 |
| F. 100% C <sub>8</sub> oxo adipate                              | 2.79                   | 6,460  |
| G. 95% C <sub>8</sub> oxo adipate+5% complex adipate B (7 cs.)  | 2.90                   | 6,780  |
| H. 90% C <sub>8</sub> oxo adipate+10% complex adipate B (7 cs.) | 2.99                   | 7,005  |
| I. 85% C <sub>8</sub> oxo adipate+15% complex adipate B (7 cs.) | 3.15                   | 7,750  |
| J. 80% C <sub>8</sub> oxo adipate+20% complex adipate B (7 cs.) | 3.27                   | 9,460  |
| K. 70% C <sub>8</sub> oxo adipate+30% complex adipate B (7 cs.) | 3.58                   | 13,300 |
| L. 100% di-isooctyl azelate                                     | 3.45                   | 8,475  |
| M. 95% di-isooctyl azelate+5% complex adipate B (7 cs.)         | 3.55                   | 9,130  |
| N. 90% di-isooctyl azelate+10% complex adipate B (7 cs.)        | 3.69                   | 10,330 |
| O. 85% di-isooctyl azelate+15% complex adipate B (7 cs.)        | 3.81                   | 12,040 |
| P. 80% di-isooctyl azelate+20% complex adipate B (7 cs.)        | 3.94                   | 14,615 |

It will be noted that about 20% ± 5% complex ester will generally bring the viscosity of the base blend to the desired level of about 12,000–12,500 cs. at -65° F. Because of the thickening effect of still other components or additives, the amount of complex esters incorporated will generally be less than about 10%. It is to be mentioned that the complex ester itself will carry considerably more load than any of the conventional diesters. As shown below, this is reflected in the base blend which has a slightly better load carrying ability than the diester alone. It is therefore advantageous to incorporate the maximum amount of complex ester providing a satisfactory low temperature viscosity can be maintained.

30 It is apparent from the above data that a blend from which the oxidation inhibitor is eliminated will show very poor oxidation-corrosion resistance. Although the above oxidation/corrosion tests were carried out at 250° F., the current test requirement calls for 347° F. At this temperature the oxidative degradation of the inhibited materials is essentially the same as above. The uninhibited materials, however, readily degrade to solid masses. As is stated above, the low molecular weight 35 dimethyl silicone polymer is operable in the concept of this invention only within restricted molecular weight ranges. This molecular weight range corresponds to a viscosity in centistokes at 25° C. of between about 3 and about 20. The data set out below show that as the 40 molecular weight increases above about the 20 cs. level, the silicone polymer becomes more and more insoluble in the base blend and hazy solutions result. It is also to be seen that when the molecular weight of the silicone polymer decreases to below about the 3 cs. viscosity level, the flash point of the resulting composition is seriously 45 lowered. The extent of the flash point lowering will of course depend largely upon the concentration of silicone employed. Because of the high volatility of the low molecular weight silicones, high concentrations will effect 50 greater flash point lowerings. This is illustrated below with a 5 cs. silicone.

Table A

| Material                                     | Flash, ° F. | Appearance at room temperature |
|----------------------------------------------|-------------|--------------------------------|
| Blend O <sup>1</sup>                         | 420         | Clear                          |
| 99% blend O <sup>1</sup> +1% 5 cs. silicone  | 415         | Do                             |
| 98% blend O <sup>1</sup> +2% 5 cs. silicone  | 425         | Do                             |
| 97% blend O <sup>1</sup> +3% 5 cs. silicone  | 405         | Do                             |
| 96% blend O <sup>1</sup> +4% 5 cs. silicone  | 390         | Do                             |
| 95% blend O <sup>1</sup> +5% 5 cs. silicone  | 380         | Do                             |
| 90% blend O <sup>1</sup> +10% 5 cs. silicone | 365         | Do                             |
| 85% blend O <sup>1</sup> +15% 5 cs. silicone | 350         | Do                             |
| 100% 5 cs. silicone                          | 310         | Do                             |

<sup>1</sup> 85% diisooctyl azelate+15% adipate complex ester B.

Load carrying ability of ester blends; parts by weight

| Base blend                     | 100<br>(100)           | 100                    | 0              | 100<br>(95)<br>(5)     | 100<br>(95)<br>(5)         | 100<br>(100)               |
|--------------------------------|------------------------|------------------------|----------------|------------------------|----------------------------|----------------------------|
| Diester (vol. percent)         |                        |                        |                |                        |                            |                            |
| Complex ester (vol. percent)   |                        | (100)                  |                |                        |                            |                            |
| Silicone                       |                        |                        | 100            |                        |                            |                            |
| Ryder gear test load, lbs./in. | 1,500/1,700<br>400/500 | 3,000/4,000<br>750/800 | 300/500<br>100 | 1,800/2,200<br>450/550 | 3,000/4,000<br>1,050/1,300 | 2,500/3,500<br>1,000/1,200 |
| SAE-SOD test load, lbs.        |                        |                        |                |                        |                            |                            |

The inclusion of a minor amount of an oxidation inhibitor such as purified phenothiazine in the base oil blend of the compositions of this invention is necessary to prevent oxidative degradation during the life of the lubricant. The stabilizing effect of phenothiazine on the diester component is readily seen in the following examples. Its effect on the diester-complex ester bases of this invention is similar. It will be noted that with phenothiazine present, metal corrosion, solidification and acidity are held to a satisfactory level. Oxygen adsorption is also nil.

75 The effect of silicone viscosity at silicone concentra-

tion of 4% on flash point and on low temperature appearance of the blend is also shown below:

Table B

| Blend                      | Flash,<br>° F. | Appearance at ° F.       |               |
|----------------------------|----------------|--------------------------|---------------|
|                            |                | 75                       | -65           |
| Base (for blend 2, page 9) | 480            | Clear                    | Clear         |
| Base+4% 1 cs. silicone     | 405            | do                       | Do            |
| Base+4% 2 cs. silicone     | 400            | do                       | Do            |
| Base+4% 3 cs. silicone     | 410            | do                       | Do            |
| Base+4% 5 cs. silicone     | 415            | do                       | Slight cloud. |
| Base+4% 10 cs. silicone    | 430            | do                       | Do            |
| Base+4% 20 cs. silicone    | 435            | do                       | Cloudy.       |
| Base+4% 50 cs. silicone    | 460            | Partial separa-<br>tion. | Separation.   |
| Base+4% 100 cs. silicone   | 465            | Incompatible             | Incompatible. |

Formulations containing the base compositions of this invention and the low molecular weight silicone polymer exhibit surprising and unexpected foaming tendencies. This effect is contrary to the teaching of the prior art which disclose silicone polymers as anti-foamants. To correct this undesirable foaming, a very small amount (0.0001 to 0.01, preferably 0.001 to .005 wt. percent) of a high molecular weight dimethyl silicone polymer (10,000 to 1,000,000, preferably 60,000 to 200,000 cs. at 25° C.) added to the blend. Data set out below show the corrective action of this additive.

Table C

|                                                                                    | MIL-L-7808 foam test                     |       |                                           |       |                                          |       |
|------------------------------------------------------------------------------------|------------------------------------------|-------|-------------------------------------------|-------|------------------------------------------|-------|
|                                                                                    | 75° F. sequence<br>1 foam volume,<br>cc. |       | 200° F. sequence<br>2 foam volume,<br>cc. |       | 75° F. sequence<br>3 foam volume,<br>cc. |       |
|                                                                                    | Blow-<br>ing                             | Final | Blow-<br>ing                              | Final | Blow-<br>ing                             | Final |
| MIL-L-7808                                                                         | 100                                      | 0     | 25                                        | 0     | 100                                      | 0     |
| Base (similar to<br>blend 2 base)                                                  | 235                                      | 0     | 40                                        | 0     | 260                                      | 0     |
| Base+0.001% DC-<br>200 60,000 cs.<br>silicone                                      | 200                                      | 0     | 35                                        | 0     | 210                                      | 0     |
| Base+0.002% DC-<br>200 60,000 cs.<br>silicone                                      | 130                                      | 0     | 20                                        | 0     | 100                                      | 0     |
| Base+0.004% DC-<br>200 60,000 cs.<br>silicone                                      | 30                                       | 0     | 15                                        | 0     | 30                                       | 0     |
| Base+0.005% DC-<br>200 60,000 cs.<br>silicone                                      | 20                                       | 0     | 10                                        | 0     | 20                                       | 0     |
| Base+0.01% DC-<br>200 60,000 cs.<br>silicone                                       | 15                                       | 0     | 10                                        | 0     | 15                                       | 0     |
| Base+0.02% DC-<br>200 60,000 cs.<br>silicone                                       | 10                                       | 0     | 10                                        | 0     | 15                                       | 0     |
| Base+0.005% DC-<br>200 10,000 cs.<br>silicone                                      | 20                                       | 0     | 15                                        | 0     | 20                                       | 0     |
| Base+0.005% DC-<br>200 200,000 cs.<br>silicone                                     | 20                                       | 0     | 10                                        | 0     | 20                                       | 0     |
| Base+0.005% DC-<br>200 500,000 cs.<br>silicone (slightly<br>insoluble)             | 30                                       | 0     | 20                                        | 0     | 50                                       | 0     |
| Base+0.005% DC-<br>200 1,000,000 cs.<br>silicone (some-<br>what incompat-<br>ible) | 40                                       | 0     | 15                                        | 0     | 50                                       | 0     |

The effect of the low molecular weight silicone polymer on the load-carrying ability of the base composition of this invention is most unusual since the base composition and especially the silicone separately are by comparison poor lubricants. The exact mechanism by which this phenomenon occurs is not clearly understood, but it

is believed that in bulk the silicone molecules assume a helical configuration which possess little adhesion to metal bearing surfaces while in solution such as in the base composition of this invention the silicone molecules uncoil, in which state the silicone possesses considerably greater energy of adhesion resulting in a closely packed oriented film on the metal bearing surfaces. Data showing the excellent lubricating properties of the base composition containing low concentrations of silicone polymers are given

in the table below. It will be seen from an examination of Table D that as the silicone polymer content of the blend is increased, the load-carrying qualities of the composition reach a maximum point and then rapidly decrease until substantially no improvement is shown. This extreme-pressure resisting characteristic is shown in both the well known SAE-SOD test loading procedure and the Shell 4-Ball E.P. test. This data is also graphically presented in Figures I and II of the accompanying drawing. It will be seen both from Table D below and the drawings

that optimum extreme pressure resistance is obtained by blends containing from about 10 to about 20 wt. percent of the low molecular weight silicone polymer. In this range apparently the dimethyl silicone molecules possess their maximum energy of adhesion.

25

Table D  
LOAD CARRYING ABILITY VS. SILICONE CONTENT OF  
ESTER BLENDS

|                                         | SAE-SOD<br>test load,<br>lbs. to<br>bearing<br>scuff | Shell 4-ball<br>EP test<br>(10 sec.),<br>min. scuff<br>load, kg. |
|-----------------------------------------|------------------------------------------------------|------------------------------------------------------------------|
|                                         |                                                      |                                                                  |
| 35                                      |                                                      |                                                                  |
| 100% base (for blend 1, page 9)         | 475                                                  | 55                                                               |
| 99% base+1% dimethyl silicone (10 cs.)  | 700                                                  | 45                                                               |
| 98% base+2% dimethyl silicone (10 cs.)  | 750                                                  | 70                                                               |
| 97% base+3% dimethyl silicone (10 cs.)  | 950                                                  | 80                                                               |
| 96% base+4% dimethyl silicone (10 cs.)  | 1,025                                                | 96                                                               |
| 95% base+5% dimethyl silicone (10 cs.)  | 1,050                                                | 108, 114                                                         |
| 90% base+10% dimethyl silicone (10 cs.) | 1,450                                                | 108                                                              |
| 85% base+15% dimethyl silicone (10 cs.) | 2,000                                                | 110                                                              |
| 80% base+20% dimethyl silicone (10 cs.) | 1,950                                                | 136, 150                                                         |
| 75% base+25% dimethyl silicone (10 cs.) | 1,800                                                | 117                                                              |
| 50% base+50% dimethyl silicone (10 cs.) | 600                                                  | 78                                                               |
| 0% base+100% dimethyl silicone (10 cs.) | 100                                                  | 24                                                               |

It will be understood that other additives such as rust inhibitors, detergents, V.I. improvers, auxiliary load carrying agents, etc. can be added to the present compositions.

It has also been found and forms another object of this invention that the synthetic lubricating compositions as set out in detail above may be utilized in the preparation of high pressure lubricating grease compositions. These lubricating greases are prepared by thickening the synthetic lubricants above to a grease consistency with a grease-forming soap.

More particularly, the present lubricating grease compositions comprise (1) about 15 to 30% by weight of a grease thickener and (2) about 70 to 85% by weight of a blend of (a) about 10 to 20% by weight of dimethyl silicone polymer having a viscosity at 25° C. of about 3 to 20 centistokes and (b) about 80 to 90% by weight of a dialkyl ester of a dicarboxylic acid having the formula:



wherein R represents a branched chain alkyl group containing 6 to 10 carbon atoms and n is an integer from 2 to 8. A particularly preferred dialkyl ester is diisooctyl azelate. The soap thickener may be a grease-forming metal soap or a grease-forming metal soap-salt complex of a metal soap of a carboxylic acid and metal salt of a carboxylic acid. Preferred metals are the alkaline earth metals, and preferred molar proportions of salt to soap are in the range of about 3.5:1 to 20:1. The soap thickeners utilized in the formulation of the grease compositions of

70

this aspect of the invention are preferably lithium stearate or a complex formed from the calcium salt of acetic acid and the calcium soap of commercial caprylic acid.

Samples of the grease compositions of this invention are set out in detail below:

## EXAMPLE I

| Formulation (percent weight)                                                     | A     | B     |
|----------------------------------------------------------------------------------|-------|-------|
| Lithium stearate                                                                 | 18.1  | 18.1  |
| Disooctyl azelate                                                                | 80.0  | ----- |
| Blend of 15% dimethyl silicone polymer (10 cs./25° C.) and 85% disooctyl azelate | ----- | 80.0  |
| Zinc naphthenate                                                                 | 0.5   | 0.5   |
| Phenyl alpha naphthylamine                                                       | 0.5   | 0.5   |
| Color stabilizer (disobutyl phenol-formaldehyde ammonia polymer)                 | 0.9   | 0.9   |
|                                                                                  | 100.0 | 100.0 |

**Preparation.**—The same procedure was used in both samples A and B. The dry preformed lithium soap was slurred in the ester or ester-blend and heated to 410° F. while stirring. The other ingredients (inhibitors) were then added and the molten grease was poured in shallow layers in pans for quick cooling. (Other rapid cooling means may be employed as long as the grease remains quiescent during passage through transition point.) The cold grease was returned to kettle, stirred to required penetration and milled or homogenized, filtered and packaged.

| Properties                                                                           | Non-silicone blend A | Silicone containing blend B |
|--------------------------------------------------------------------------------------|----------------------|-----------------------------|
| Appearance                                                                           | Excellent            | Excellent                   |
| Dropping point, °F.                                                                  | 360                  | 360                         |
| Penetrations, 77° F. mm./10:                                                         |                      |                             |
| Unworked                                                                             | 285                  | 285                         |
| Worked, 60 strokes                                                                   | 295                  | 295                         |
| Worked, 100,000 strokes                                                              | 342                  | 342                         |
| Low temp. performance, -65° F., time to turn a 204 bearing under 2,000 gram-cm. load | (1)                  | (1)                         |
| Load carrying performance in Shell 4-ball E.P. test:                                 |                      |                             |
| Scar diameter at given load, mm.                                                     |                      |                             |
| 32 kg.                                                                               | 0.36                 | 0.26                        |
| 40 kg.                                                                               | 0.50                 | 0.28                        |
| 50 kg.                                                                               | 0.75                 | 0.30                        |
| 63 kg.                                                                               | 1.00                 | 0.32                        |
| 79 kg.                                                                               | 1.79                 | 0.37                        |
| 100 kg.                                                                              | 2.00                 | 0.38                        |
| 126 kg.                                                                              | Weld                 | Weld                        |
| Average 3 balls measured in 2 directions                                             |                      |                             |

<sup>1</sup> Less than 5 secs.

<sup>2</sup> Up to and including this load there was no scuff or film rupture.

## EXAMPLE II

| Formulation (percent weight)                                                     | C     | D     |
|----------------------------------------------------------------------------------|-------|-------|
| Acetic acid                                                                      | 12.0  | 12.0  |
| Commercial caprylic acid <sup>1</sup>                                            | 6.0   | 6.0   |
| Hydrated lime                                                                    | 9.8   | 9.8   |
| Phenyl naphthylamine                                                             | 1.0   | 1.0   |
| Blend of 15% dimethyl silicone polymer (10 cs./25° C.) and 85% disooctyl azelate | 71.2  | ----- |
| Disooctyl azelate                                                                | 71.2  | ----- |
|                                                                                  | 100.0 | 100.0 |

<sup>1</sup> 18% lauric, 58% capric, 24% caprylic (Sap. No. 324).

**Preparation.**—The lime and ester or ester-silicone blend was charged to a fire heated kettle and heated to 135° F. A blend of acetic and caprylic acids was then added and heating continued to 500° F. The heat was then shut off and the mass cooled to 200° F. where phenyl alpha naphthylamine was added and the grease further cooled to 150° F. At that temperature the grease was homogenized and packaged.

| Properties                                             |      | Non-Silicone Blend C | Silicone Containing Blend D |
|--------------------------------------------------------|------|----------------------|-----------------------------|
| Appearance                                             |      | Excellent            | Excellent                   |
| Dropping point, °F.                                    | 500+ | 500+                 | 500+                        |
| Penetrations, 77° F. mm./10:                           |      |                      |                             |
| Unworked                                               | 275  | 275                  | 275                         |
| Worked, 60 strokes                                     | 280  | 280                  | 280                         |
| Worked, 100,000 strokes                                | 325  | 325                  | 325                         |
| 10 Extreme pressure properties:                        |      |                      |                             |
| Shell 4-ball test scar diameters at given load in mm.— |      |                      |                             |
| 32 kg.                                                 | 0.28 | 0.28                 | 0.28                        |
| 40 kg.                                                 | 0.29 | 0.30                 | 0.30                        |
| 50 kg.                                                 | 0.31 | 0.30                 | 0.33                        |
| 63 kg.                                                 | 0.38 | 0.33                 | 0.33                        |
| 79 kg.                                                 | 0.47 | 0.37                 | 0.37                        |
| 100 kg.                                                | 0.72 | 0.40                 | 0.40                        |
| 126 kg.                                                | 0.90 | 0.44                 | 0.44                        |
| 160 kg.                                                | 1.25 | 0.49                 | 0.49                        |
| 200 kg.                                                | 1.30 | 0.95                 | 0.95                        |
| 251 kg.                                                | 2.20 | 1.10                 | 1.10                        |
| 316 kg.                                                | Weld | 2.50                 | 2.50                        |
| E.P. value (calculated) (based on Hertz loadings)      | 52.5 | 86.5                 |                             |

<sup>1</sup> Up to this point inclusive there was no apparent scuff or film rupture.

What is claimed is:

1. A fluid synthetic lubricating composition having improved extreme pressure resisting characteristics consisting essentially of (1) a major proportion of a lubricating oil base consisting of (a) 80 to 99% by volume of a dialkyl ester of a dicarboxylic acid having the formula:



wherein R represents a branched chain alkyl group containing 6 to 10 carbon atoms and n is an integer from 2 to 8 and (b) 1 to 20% by volume of a complex ester having the formula:



wherein R represents a branched chain alkyl group containing 6 to 10 carbon atoms, x is an integer from 2 to 8 and z is an integer from 2 to 6; (2) about 0.25 to 2% by weight, based on the lubricating oil base, of an antioxidant; (3) about 2 to 25% by weight, based on the lubricating oil base of dimethyl silicone polymer having a viscosity at 25° C. of about 3 to 20 centistokes; and (4) about 0.001 to 0.1% by weight, based on the lubricating oil base, of a second dimethyl silicone polymer having a viscosity of 25° C. of at least about 10,000 centistokes.

2. A fluid synthetic lubricating composition having improved extreme pressure resisting characteristics consisting essentially of (1) a major proportion of a lubricating oil base consisting of (a) 92 to 97% by volume of a dialkyl ester of a dicarboxylic acid having the formula:



wherein R represents a branched chain alkyl group containing 6 to 10 carbon atoms and n is an integer from 2 to 8 and (b) 3 to 8% by volume of a complex ester having the formula:



wherein R represents a branched chain alkyl group containing 6 to 10 carbon atoms, x is an integer from 2 to 8 and z is an integer from 2 to 6; (2) about 0.25 to 2% by weight, based on the lubricating oil base, of phenothiazine; (3) about 3 to 5% by weight, based on the lubricating oil base, of dimethyl silicone polymer having a viscosity at 25° C. of about 3 to 20 centistokes; and (4) about 0.001 to 0.005% by weight, based on the lubricating oil base, of a second dimethyl silicone polymer having a viscosity at 25° C. of about 60,000 to 200,000 centistokes.

3. A fluid synthetic lubricating composition having improved extreme pressure resisting characteristics consisting essentially of (1) a major proportion of a lubri-

11

cating oil base consisting of (a) 92 to 97% by volume of a dialkyl ester of a dicarboxylic acid having the formula:



wherein R represents a branched chain alkyl group containing 6 to 10 carbon atoms and n is an integer from 2 to 8 and (b) 3 to 8% by volume of a complex ester having the formula:



wherein R represents a branched chain alkyl group containing 6 to 10 carbon atoms, x is an integer from 2 to 8 and z is an integer from 2 to 6; (2) about 0.25 to 2% by weight, based on the lubricating oil base, of phenothiazine; (3) about 5 to 20% by weight, based on the lubricating oil base, of dimethyl silicone polymer having a viscosity at 25° C. of about 3 to 20 centistokes; and (4) about 0.001 to 0.005% by weight, based on the lubricating oil base, of a second dimethyl silicone polymer having a viscosity at 25° C. of about 60,000 to 200,000 centistokes.

4. A fluid synthetic lubricating composition having improved extreme pressure resisting characteristics consisting essentially of (1) a major proportion of a lubricating oil base consisting of (a) about 95% by volume of diisooctyl azelate and (b) about 5% of a complex ester of 1 mol of tetraethylene glycol with 2 mols of sebacic acid and 2 mols of 2-ethyl hexanol; (2) about 1% by weight, based on the lubricating oil base, of phenothiazine; (3) about 5% by weight, based on the lubricating oil base, of dimethyl silicone polymer having a viscosity at 25° C. of about 10 centistokes; and (4) about 0.001% by weight, based on the lubricating oil base, of dimethyl silicone polymer having a viscosity at 25° C. of about 60,000 centistokes.

5. A fluid synthetic lubricating composition having improved extreme pressure resisting characteristics con-

12

sisting essentially of (1) a major proportion of a lubricating oil base consisting of (a) 97% by volume of 2-ethyl hexyl sebacate and (b) about 3% by volume of complex ester of 1 mol of tetraethylene glycol with 2

5 mols of adipic acid and 2 mols of C<sub>8</sub> branched chain primary alcohol; (2) about 1% by weight, based on the lubricating oil base, of phenothiazine; (3) 4% by weight, based on the lubricating oil base, of dimethyl silicone polymer having a viscosity at 25° C. of about 10 centistokes; (4) about 0.001% by weight, based on the lubricating oil base, of dimethyl silicone polymer having a viscosity at 25° C. of about 60,000 centistokes; and (5) about 1% by weight, based on the lubricating oil base, of tricresyl phosphate.

10 6. A fluid synthetic lubricating composition having improved extreme pressure resisting characteristics consisting essentially of (1) a major proportion of a lubricating oil base consisting of (a) about 38% by volume of C<sub>8</sub> branched chain primary adipate, (b) about 57% by volume of C<sub>10</sub> branched chain primary adipate and (c) about

15 5% by volume of a complex ester of 1 mol tetraethylene glycol with 2 mols of adipic acid and 2 mols of C<sub>8</sub> branched chain primary alcohol; (2) about 1% by weight, based on the lubricating oil base, of phenothiazine; (3) about 5% by weight, based on the lubricating oil base, of dimethyl silicone polymer having a viscosity at 25° C. of about 10 centistokes; and (4) about 0.001% by weight, based on the lubricating oil base, of dimethyl silicone polymer having a viscosity at 25° C. of about 60,000 centistokes.

#### References Cited in the file of this patent

#### UNITED STATES PATENTS

|    |           |               |               |
|----|-----------|---------------|---------------|
| 35 | 2,407,037 | Sowa          | Sept. 3, 1946 |
|    | 2,589,317 | Young et al.  | Mar. 18, 1952 |
|    | 2,750,341 | Morway et al. | June 12, 1956 |